

## UNITED STATES PATENT OFFICE

2,114,669

TREATING TEXTILE MATERIAL AND  
PRODUCT THEREOF

George Schneider, Montclair, N. J., assignor to  
Celanese Corporation of America, a corpora-  
tion of Delaware

No Drawing. Original application June 10, 1932,  
Serial No. 616,573. Divided and this applica-  
tion December 4, 1935, Serial No. 52,829

4 Claims. (Cl. 8—2)

This invention relates to the treatment of tex-  
tile materials made of or containing organic de-  
rivatives of cellulose and relates more particu-  
larly to the treatment of such materials with hot  
aqueous fluids.

This application is a division of my applica-  
tion Serial No. 616,573 filed June 10, 1932, now  
Patent No. 2,041,868, patented May 26, 1936.

An object of my invention is to protect tex-  
tile materials comprising organic derivatives of  
cellulose against impairment of desirable prop-  
erties when subjected to hot aqueous fluids. A  
further object of my invention is to diminish or  
prevent the tendency of pile of organic derivative  
of cellulose yarn to agglomerate when fabric  
having a pile of organic derivative of cellulose  
yarn is subjected to hot aqueous liquids. Other  
objects of this invention will appear from the  
following detailed description.

Fabrics having a pile made of yarn of cellu-  
lose acetate or other organic derivative of cellu-  
lose present serious difficulties when subjected  
to finishing treatments such as dyeing, scouring,  
degumming, etc. which involve treatment with  
hot aqueous liquids. I have found that when  
such fabrics are treated with hot aqueous liquids,  
the pile yarns tend to agglomerate into tufts,  
with the result that the appearance of the fabric  
is not uniform and the value of the fabric is  
greatly impaired through the lack of uniform  
lustre or sheen demanded of velvets or other pile  
fabrics.

I have found that if readily ionizable salts are  
present while such pile fabrics are treated with  
hot aqueous fluids the agglomeration of the or-  
ganic derivative of cellulose pile yarn into tufts  
is avoided, thus making possible the finishing of  
fabric made of organic derivative of cellulose  
pile to form a fabric having substantially uni-  
form sheen.

I have further found that if such neutral salts  
are present in a bath employed to degum the nat-  
ural silk in a mixed fabric containing both or-  
ganic derivative of cellulose yarn and natural  
silk yarn, they protect the organic derivative of  
cellulose yarn against the deleterious action of  
the hot soap solutions employed for the de-  
gumming.

In accordance with one aspect of my invention,  
I treat fabrics containing both yarns of organic  
derivative of cellulose and natural silk yarns in  
the gum at elevated temperatures with a de-  
gumming bath containing a readily ionizable salt  
or other compound. In accordance with another  
aspect of my invention, I treat fabric having a

pile made of yarns of organic derivative of cel-  
lulose with hot aqueous baths containing such  
salts or compounds, in order to avoid the ag-  
glomeration of the pile into tufts.

The textile material may contain or be made 5  
of any suitable organic derivative of cellulose  
such as organic esters of cellulose and cellulose  
ethers. Examples of organic esters of cellulose  
are cellulose acetate, cellulose formate, cellulose  
propionate and cellulose butyrate, while examples 10  
of cellulose ethers are ethyl cellulose, methyl cel-  
lulose and benzyl cellulose. This invention how-  
ever will be described more specifically in connec-  
tion with the treatment of textile materials made  
of or containing the acetone-soluble type of cel- 15  
lulose acetate. If an acetone-soluble cellulose  
acetate of relatively high acetyl value, say 57 to  
59% determined as acetic acid, is employed in  
making the textile material, particularly good  
results are obtained due to the greater resistance 20  
of such cellulose acetate to the agglomerating ac-  
tion of hot aqueous liquids.

The degumming bath employed may be the  
usual soap solutions used for this purpose and  
usually the temperature of degumming will be on 25  
the order of 90 to 100° C.

Any suitable readily ionizable salt may be em-  
ployed to prevent agglomeration of the organic  
derivative of cellulose yarn. Examples of such  
salts are the sulfates, chlorides, nitrates, chro- 30  
mates and acetates of sodium, potassium, magne-  
sium, ammonium or aluminum. The amount of  
these salts present will vary with the specific  
salt used, the temperature of treatment and other  
considerations. Generally the salts will be pres- 35  
ent in the aqueous liquid in a concentration of  
0.5 to 10%. Materials other than salts may be  
used for this purpose, an example of which is cane  
sugar.

Since the ionizable salts tend to reduce the 40  
alkalinity of the soap solutions used for degum-  
ming and therefore diminish the power of the  
bath to degum the natural silk, I prefer to add  
such an amount of alkali or alkaline salt to the  
soap solution containing these salts as to impart 45  
to it the degree of alkalinity of soap baths ordi-  
narily used for degumming natural silk and hav-  
ing a pH value of above 8 and preferably below  
10, when yarns of cellulose acetate or other or-  
ganic esters of cellulose are present and it is de- 50  
sired to avoid substantial saponification of the  
same. By raising the degree of alkalinity of the  
degumming bath in this manner, the time re-  
quired for degumming is reduced. Alkalies or  
strongly alkaline salts such as sodium hydroxide, 55

potassium hydroxide, sodium carbonate or potassium carbonate may be used for this purpose, but in order to render possible a more delicate control of the alkalinity, I prefer to use less strongly 5 alkaline salts such as disodium phosphate, dipotassium phosphate or borax.

The treatment of pile fabric such as velvets by subjecting the same to hot finishing baths, such as are employed in dyeing, scouring, degumming, 10 etc., that contain these salts or substances is of great importance not only in the case where degumming of the natural silk yarn present in the backing of such fabric is to occur, but is of importance in the treatments of all kinds of fabric 15 having a pile of organic derivative of cellulose yarn, whether the backing is also made of organic derivative of cellulose or whether it is made of silk, cotton, regenerated cellulose, wool or any other fibres. The presence of these salts prevents 20 the agglomeration of the pile into tufts and consequent formation of "bald" spots in such fabric.

In order further to illustrate my invention, but without being limited thereto, the following specific examples are given.

*Example I*

This example is given as illustrating the use of my invention for both degumming natural silk 30 in a mixed natural silk and cellulose acetate fabric and also for protecting the cellulose acetate pile against agglomeration.

A degumming bath is made up containing:

|                                                 | Grams per litre |
|-------------------------------------------------|-----------------|
| 35 Olive oil soap                               | 50              |
| Disodium phosphate ( $Na_2HPO_4 \cdot 12H_2O$ ) | 25              |
| Sodium sulfate (anhydrous)                      | 25              |

A velvet having a pile made of yarn of acetone-soluble cellulose acetate and a back of natural silk in the gum is treated with this degumming bath at a temperature of 93 to 100° C., say 95° C., for 1½ to 2½ hours. The fabric is then subjected to any desired finishing treatment such as 40 washing, dyeing, steaming, etc. The silk is completely degummed, and yet the cellulose acetate pile is free of agglomeration and the fabric presents a uniform lustre or sheen.

*Example II*

50 This example is also given to illustrate the use of my invention both for degumming natural silk in a mixed natural silk cellulose acetate fabric

and for protecting the cellulose acetate pile against agglomeration.

A degumming bath is made up containing:

|                | Grams per litre | 5 |
|----------------|-----------------|---|
| Olive oil soap | 50              | 5 |
| Cane sugar     | 50              |   |

A velvet having a pile made of yarn of acetone-soluble cellulose acetate and a back of natural silk in the gum is treated with this degumming bath at a temperature of about 95° C. for 1 to 2 hours. The fabric is then subjected to any desired finishing treatment such as washing, dyeing, steaming, etc. The silk is completely degummed, and the cellulose acetate pile is free of agglomeration and the fabric presents a uniform lustre or sheen. 15

It is to be understood that the foregoing detailed description is given merely by way of illustration and that many variations may be made therein without departing from the spirit of my 20 invention.

Having described my invention, what I desire to secure by Letters Patent is:

1. Process of degumming natural silk contained in a pile fabric which comprises subjecting a fabric having a back containing natural silk yarn and a pile containing organic derivative of cellulose yarn to the action of a hot degumming bath, which bath contains sugar in a concentration of at least 0.5%. 25

2. Process of degumming natural silk contained in a pile fabric which comprises subjecting a fabric having a back containing natural silk yarn and a pile containing cellulose acetate yarn to the action of a hot degumming bath, 35 which bath contains sugar in a concentration of at least 0.5%.

3. In the method of treating a pile fabric having a pile comprising yarns of organic derivative of cellulose wherein the fabric is subjected to a 40 hot aqueous fluid, the step of inhibiting the agglomeration of the organic derivative of cellulose pile yarn by treating the fabric with an aqueous fluid containing sugar in a concentration of at least 0.5%. 45

4. In the method of treating a pile fabric having a pile comprising yarns of cellulose acetate wherein the fabric is subjected to a hot aqueous fluid, the step of inhibiting the agglomeration of the cellulose acetate pile yarn by treating the 50 fabric with an aqueous fluid containing sugar in a concentration of at least 0.5%.

GEORGE SCHNEIDER.